

## UNITED STATES PATENT OFFICE

2,247,042

## EXTREME PRESSURE LUBRICANT

Henry G. Berger and Darwin E. Badertscher,  
Woodbury, and Francis M. Seger, Pitman, N. J.,  
assignors to Socony-Vacuum Oil Company, In-  
corporated, New York, N. Y., a corporation of  
New York

No Drawing. Application September 25, 1940,  
Serial No. 358,236

8 Claims. (Cl. 252—48)

This invention, which is a continuation in part of that disclosed in our copending application Serial No. 177,891, filed December 3, 1937, relates to lubricant compositions adapted for use as extreme pressure lubricants.

As is well known to those familiar with the art, the ordinary type of hydrocarbon lubricant comprised only of a petroleum fraction is incapable of withstanding the enormous pressures encountered between engaged surfaces in various types of modern machinery such as the hypoid gears used in motor vehicles. This fact has led to the development of the so-called extreme pressure lubricant, which is comprised of a suitable carrying medium such as a viscous mineral oil fraction and a minor proportion of an addition agent which under the extreme pressure conditions encountered will provide or form between the engaged surfaces a lubricant film capable of withstanding these high pressures.

Ingredients of the type just referred to are known as extreme pressure agents or E. P. bases, and numerous materials have been proposed for such use. Among the various extreme pressure agents which have been proposed and which have met with varying degrees of success are oil-soluble organic materials which contain sulfur and chlorine. Our present invention is related to this general type of compound.

For the purpose of testing the efficacy of materials as extreme pressure agents, it is customary to prepare mineral oil blends containing a minor proportion of the agent to be tested and subject the oil blank and the blend to one or more of the various laboratory tests which have been devised to give an indication of the load-carrying capacity of such lubricants. Typical tests recognized in the art as being satisfactory for this purpose are the Almen pin test described by Wolfe and Mougey, Proc. A. P. I. 1932, pages 118-130, and the S. A. E. test described in S. A. E. Journal 39, 23-4 (1936).

The aforesaid copending application Serial No. 177,891 discloses as extreme pressure agents the general class of compounds or reaction products obtained by reacting perchloromethylmercaptan with organic compounds containing replaceable hydrogen or replaceable metal atoms. The present invention is concerned with a specific group of reaction products falling into that general class, namely, the products obtained by reacting perchloromethylmercaptan with organic amines.

Perchloromethylmercaptan is the chlorinated substituted sulfur chloride having the formula  $\text{CSCl}_4$  or  $\text{Cl}_3\text{C}-\text{SCl}$ . It can be prepared by the

chlorination of carbon disulfide according to the method of Helfrich and Reid (Journal American Chemical Society, 43, 591 (1921)). For example, carbon disulfide containing about 0.4 per cent by weight of iodine was chlorinated in the absence of direct sunlight at a temperature maintained below 25° C. until the volume of the reaction mixture had doubled. The crude reaction product, which contains carbon tetrachloride and sulfur chlorides in addition to perchloromethylmercaptan, can be used in the preparation of the reaction products contemplated by this invention, but it is preferable to purify the crude product by distillation on a water bath at about 100° C., followed by steam distillation. Subsequent vacuum-distillation of the material refined in this manner indicated that the steam-distilled material was practically pure.

For the organic amines contemplated herein to obtain reaction products for use as extreme pressure agents, preference is given to the primary and secondary amines. These amines may be aliphatic amines such as mono- or di- ethyl amine, mono- or di- propyl amine, mono- or di- butyl amine, mono- or di- cyclohexyl amine, or they may be aromatic amines such as aniline and its derivatives, naphthylamine and its derivatives, etc.

The procedures which may be followed in synthesizing reaction products of the type contemplated herein as extreme pressure agents may be obtained from the following examples describing typical preparations. In these examples we have also given the results of extreme pressure tests showing the effectiveness of these illustrative products in improving the extreme pressure characteristics of a typical mineral oil.

## EXAMPLE ONE

40 *Reaction products of perchloromethylmercaptan and monobutyl amine*

The reaction mixture was prepared by dissolving 93 grams (0.5 mole) of perchloromethylmercaptan and 37 grams (0.5 mole) of monobutylamine in separate portions of petroleum ether, after which the amine solution was stirred with an aqueous solution of 29 grams (0.273 mole or 0.54 equivalent) of sodium carbonate while the perchloromethylmercaptan solution was added thereto. The addition was made at an average temperature of about 10° C., and the rate of addition was such that it consumed about 40 minutes. The petroleum ether solution of the product was washed and filtered and the solvent removed by

placing under a vacuum of approximately 30 mm. at room temperature. The final product obtained was a red-brown liquid of low viscosity and a characteristic somewhat sweet odor. The yield was approximately 105 grams. A mineral oil blend containing 5 per cent of this product passed the S. A. E. test at a load of 580+, the machine operating at a speed of 1000 R. P. M. with a 14.6:1 rubbing ratio and a loading rate of 8.35 pounds per second. The 5 per cent mineral oil blend of this product went to a load of 26,000 pounds in the Almen pin test before failure.

EXAMPLE Two

Reaction product of perchloromethylmercaptan and dibutylamine

In this preparation 37.2 grams (0.2 mole) of perchloromethylmercaptan and 51.6 grams (0.4 mole) of dibutylamine were reacted together in a benzol solution. The hydrochloride formed was filtered out; the benzol solution of the product was water-washed and topped, yielding a dark brown residual liquid which was finally filtered. The final yield of the product thus obtained was 45.5 grams. A 5 per cent blend of this product in mineral oil failed in the S. A. E. test at 350 pounds and in the Almen pin test went to 30,000 pounds without failure.

EXAMPLE THREE

Reaction product of perchloromethylmercaptan and dicyclohexylamine

In this preparation 51 grams (0.27 mole) of perchloromethylmercaptan and 100 grams (0.55 mole) of dicyclohexylamine were reacted in benzol solution. The hydrochloride formed was removed by filtration and the benzol solution topped off to yield a solid residue. A 5 per cent blend of this product in the same mineral oil described in connection with Example One failed the S. A. E. test at a load of 295 pounds.

EXAMPLE FOUR

Reaction product of perchloromethylmercaptan and ethyl aniline

A petroleum ether solution containing 61 grams (0.5 mole) of ethyl aniline was prepared and mixed with an aqueous solution containing an excess of sodium carbonate. While stirring this solution a petroleum ether solution containing 93 grams (0.5 mole) of perchloromethylmercaptan was added over a period of about 25 minutes during which the temperature of the reaction mixture was maintained at a temperature of 8° C. The petroleum ether solution containing the reaction product was washed with water, filtered and the solvent removed at room temperature by means of vacuum.

The product obtained after filtering was a light amber liquid of low viscosity and mild odor. The yield was 116 grams. A 5 per cent blend of this product in the mineral oil described in connection with Example One failed in the S. A. E. test at a load of 290 pounds and the Almen pin test at a load of 26,000 pounds.

The blank oil used in the foregoing examples

failed in the S. A. E. test at a load of 20 pounds and in the Almen pin test at a load of 3000 pounds.

The reaction products contemplated herein may be blended with mineral oil fractions or other suitable carrying agents in amounts ranging from 0.5 per cent to 20 per cent to provide lubricants for use under extreme pressure conditions. It is to be understood that while the foregoing examples describe specific reaction procedures and specific amines for the secondary reactants, the invention is not limited to such specific procedural details nor to specific amines but includes within its scope such changes as fairly come within the spirit of the appended claims.

We claim:

1. An extreme pressure lubricant comprising a hydrocarbon lubricating oil and in admixture therewith a minor proportion of the product obtained by the reaction of perchloromethylmercaptan with an organic amine.

2. An extreme pressure lubricant comprising a hydrocarbon lubricating oil and in admixture therewith a minor proportion of the product obtained by the reaction of perchloromethylmercaptan with a primary organic amine.

3. An extreme pressure lubricant comprising a hydrocarbon lubricating oil and in admixture therewith a minor proportion of the product obtained by the reaction of perchloromethylmercaptan with a secondary organic amine.

4. An extreme pressure lubricant comprising a hydrocarbon lubricating oil and in admixture therewith a minor proportion, from about 0.5 per cent to about 20 per cent, of the product obtained by the reaction of perchloromethylmercaptan with an organic amine.

5. An extreme pressure lubricant comprising a hydrocarbon lubricating oil and in admixture therewith a minor proportion, from about 0.5 per cent to about 20 per cent, of the product obtained by the reaction of perchloromethylmercaptan with a primary organic amine.

6. An extreme pressure lubricant comprising a hydrocarbon lubricating oil and in admixture therewith a minor proportion, from about 0.5 per cent to about 20 per cent, of the product obtained by the reaction of perchloromethylmercaptan with a secondary organic amine.

7. An extreme pressure lubricant comprising a hydrocarbon lubricating oil and in admixture therewith a minor proportion of the product obtained by the reaction of perchloromethylmercaptan with an organic amine, said reaction product being present in an amount sufficient to increase the load-carrying capacity of the oil.

8. An extreme pressure lubricant comprising a hydrocarbon lubricating oil and in admixture therewith a minor proportion, sufficient to increase the load-carrying capacity of the oil, of the product obtained by reacting perchloromethylmercaptan with an organic amine selected from the group of monobutyl amine, dibutyl amine, dicyclohexyl amine, and ethyl aniline.

HENRY G. BERGER,  
DARWIN E. BADERTSCHER,  
FRANCIS M. SEGER.